

Nov. 5, 1929.

H. G. WALKER

1,734,700

COATED CORE

Filed June 5, 1923



Inventor  
Howard G. Walker  
by *Alfathem*  
Atty.

## UNITED STATES PATENT OFFICE

HOWARD GEORGE WALKER, OF BERWYN, ILLINOIS, ASSIGNOR TO WESTERN ELECTRIC COMPANY, INCORPORATED, OF NEW YORK, N. Y., A CORPORATION OF NEW YORK

## COATED CORE

Application filed June 5, 1923. Serial No. 643,557.

This invention relates to improvements in coated cores, and more particularly to electrical conductors coated with an insulating material which is impervious to moisture.

5 An object of the invention is to provide an electrical conductor with an insulating material having the desirable moisture-proof qualities of rubber, and in addition one which has low dielectric losses, is flexible and sufficiently tough and durable to resist abrasion in handling.

Another object of the invention is to provide an electrical conductor with a coating of insulating material which is impervious 15 to moisture, the coating being of a type that it may be rapidly applied and including ingredients which are less expensive than the ingredients previously used in insulating materials having equivalent physical, dielectric, 20 and moisture-proofing qualities.

An article made in accordance with the present invention may comprise a core, preferably in strand form and, in cases where the finished article serves as an electrical conductor, of electrical conducting metal such as copper, coated with fibrous material which may be applied in any suitable manner. Although the fibrous material may be applied as a strand serving, as a braided covering, or 30 both, or applied in some other manner, I preferably coat the metallic core with pulp made of some cheap material such as wood, manila, jute, esparto, or hemp, but the pulp may when desired be formed of rag, cotton, linen, asbestos, etc. This pulpos material is preferably applied to the core by the method and apparatus disclosed in Patents Nos. 1,615,416 and 1,615,417, issued on January 25, 1927 to H. G. Walker et al., respectively, 35 wherein the pulpos material is held on the core solely by an intermingling of the fibers thereof. The coated core is then impregnated with rubber latex which is a product of the rubber tree containing some water, or it may be found preferable in some instances to dilute or concentrate the rubber latex prior to the impregnation of the pulpos material therewith. Ammonia may be mixed with the latex to prevent the natural coagulation thereof. 50 The impregnation may be accomplished by

immersing the coated core within a bath of the rubber latex in either its natural, diluted, or concentrated form, the core then being withdrawn from the bath and either dried at room temperature or by the application 55 of heat. It may be found desirable where this method is employed to immerse the coated core a plurality of times, drying the coating between each immersion in order to cause a thorough impregnation thereof. Other methods of impregnation may be employed as by the use of vacuum or pressure in a well known manner.

In impregnating the pulpos material with rubber latex each of the fibers of the pulpos material is saturated with the latex which 65 renders the fibers to an extent elastic. The elastic quality given the fibers and the cementing action of the rubber causes the pulpos material to resist abrasion as well as increases the flexibility of the coating.

Electrical conductors coated with pulpos material impregnated with rubber latex may be used under conditions approximating those to which ordinary rubber covered wire 75 is subjected. Conductors so coated may be used to advantage in the manufacture of telephone switchboard cable since the coating is moisture-proof, has low dielectric losses, and is tough enough to resist abrasion during 80 the handling of the cable in applying it to the switchboard.

The simplicity of the method of producing and applying the insulation to an electrical conductor, as well as the cheapness of 85 the ingredients employed, results in an electrical conductor considerably less expensive than conductors heretofore provided with an insulation having similar physical, insulating, and moisture-proof characteristics. 90

In the accompanying drawing illustrating an electrical conductor made in accordance with the invention, the reference numeral 5 indicates a strand of conducting material, preferably of copper, which is coated with 95 pulpos material preferably applied by the method and apparatus disclosed in the Walker-March patents hereinbefore referred to. The insulating material as shown in the drawing is cut away to more clearly show the 100

character thereof, and the reference numeral 10 indicates a portion of the pulpois material unimpregnated, while the reference numeral 15 indicates the said material after it has been impregnated with rubber introduced by an emulsion free from sulphur.

What is claimed is:

1. An electrical conductor comprising a metallic strand and a continuous, homogeneous, integral coating engaging the strand, consisting of felted fibrous pulp free of adhesive material impregnated with a rubber emulsion.
- 10 2. An electrical conductor comprising a metallic strand and a continuous, homogeneous, integral coating enclosing the strand, consisting solely of loosely felted and matted paper impregnated with a rubber emulsion.
- 15 3. An electrical conductor comprising a metallic strand and a continuous, homogeneous, integral, flexible coating enclosing the strand, consisting of loosely felted fibrous paper free of adhesive material impregnated with rubber introduced in an emulsion.

In witness whereof, I hereunto subscribe my name this 23 day of May A. D., 1923.

HOWARD GEORGE WALKER.

30

35

40

45

50

55

60

65